

W. W. COBLENTZ.  
ELECTRIC LIGHTING.  
APPLICATION FILED JULY 7, 1908.

1,135,663.

Patented Apr. 13, 1915.

Fig. 1.



Fig. 2.



Fig. 3.



WITNESSES:

Walter B. Emerson  
C. L. Sexton

INVENTOR

W. W. Coblenz

# UNITED STATES PATENT OFFICE.

WILLIAM WEBER COBLENTZ, OF POLAND, OHIO.

## ELECTRIC LIGHTING.

1,135,663.

Specification of Letters Patent. Patented Apr. 13, 1915.

Application filed July 7, 1908. Serial No. 442,404.

To all whom it may concern:

Be it known that I, WILLIAM WEBER COBLENTZ, a citizen of the United States, and resident of Poland, county of Mahoning, 5 State of Ohio, have invented certain new and useful Improvements in Electric Lighting, of which the following is a specification.

My invention relates to a method of and means for producing light by the incandescence of material traversed by electric currents.

The object of the invention is to cause the electric current to produce a maximum 5 amount of light with a minimum amount of heat.

When a solid conductor is traversed by an electric current, a relatively small proportion of the energy is emitted as radiant energy of wave lengths which affect the eye, while a large amount of energy is transformed into waves of such length as not to be visible but manifested as heat. All of the devices heretofore employed using solid materials for the light emitting elements, 10 under normal working conditions emit a continuous spectrum of radiant energy of which only from 3% to 5% is in the visible spectrum, the remainder being useless as far as the yielding of light is concerned. This percentage may be materially increased provided a solid conductor can be secured, which under normal working conditions emits a discontinuous or "banded" spectrum 15 in the infra-red. By continuous spectrum I mean that the spectral energy curve obtained by means of a prism transparent to heat rays and a heat measuring device, such as a bolometer or thermopile, is smooth and continuous without indentations or protuberances. The infra red emission spectrum so obtained from a rod constructed as provided by my invention even at the highest working temperatures is not smooth and 20 continuous but is deeply indented, i. e., broken into distinct bands. This results in an increase in the amount of light emitted in proportion to the amount of heat generated.

I have discovered that numerous solid 25 substances for example, certain oxids, carbonates, sulfates, etc., when heated to incandescence will emit discontinuous banded spectra in the infra red. Of these, good examples for producing light are oxid of aluminum, and fluo-silicate of aluminum (topaz). These materials are electrical

non-conductors at moderate temperature and offer great resistance to the passage of current even at high temperature.

One object of my invention is to render 60 such substances electrically conducting so as to take advantage of the discontinuous emission spectrum.

Another object of my invention is to provide incandescent bodies composed of such 65 materials with a thread of better conducting material; for example, sodium or potassium aluminum silicate, which thread is joined to the more refractory and less conducting base, such as for example, oxid of 70 aluminum.

In order to provide such a thread of better conducting material, I may for instance, attach a rod of oxid of aluminum to the current terminals by means of sodium or potassium aluminum silicate melted upon the ends of the rod and surrounding the platinum or other metallic conductor. I then place the rod in the secondary circuit of a transformer from 1000 to 2000 volts having 75 a capacity of from 100 to 300 watts, the flame from a blast lamp being allowed to play over the rod. This causes a spark discharge over the glower with the volatilization of a yellow vapor from the aluminum silicate. In a short time a narrow streak of 80 white light becomes visible along one side of the glower due to the deposition of some of the vapor and immediately the glower is rendered conducting and incandescent. The 85 glower is then ready for use and for subsequent operation is heated to a low red heat in any convenient manner, whereupon the streak becomes electrically conducting and emits an intense white light, and immediately after that the main part of the glower becomes conductive to the current and incandescent.

It is, of course, understood that in the 90 "flashing" process, lines or threads of material may be wide bands of the same, almost covering the base of aluminum oxid. It is 95 also to be understood that in the finished glower this better conducting streak is probably a chemical compound formed by the aluminum silicate and the aluminum oxid, and that it is firmly attached to the base or body of aluminum oxid.

The theory of the operation of my glower 100 is as follows: The aluminum silicate has a 105 low melting point, but in combination with the highly refractory alumina, the melting

point is raised by an unknown amount, so that the combination can be operated at a very high temperature, say from 1800 to 2000° C., without vaporizing. The base of 5 alumina becomes somewhat conducting at white heat and emits some light, but the most of the light is emitted by the complex aluminum silicate thread.

For the purpose of my invention in order 10 to produce the non-conducting base, I do not confine myself to alumina, but it is obvious that I may employ other substances or I may make such substances better electrical conductors by mixing with them in a 15 pulverized form a small amount of sodium or potassium aluminum silicate, thorium, or yttrium oxid, or any other substance suitable for increasing the conductivity, provided always that the banded emission spectrum in the infra red is not seriously affected thereby. In this case the whole glower 20 corresponds to the fine thread of better conducting material obtained by flashing a rod of alumina in the vapors of some aluminum 25 silicate.

In the practice of my invention I build up the base of aluminum oxid by softening particles of this material in a oxy-hydrogen flame and gradually adding thereto until a 30 suitable length is obtained. A glower of powdered aluminum oxid thus built up in the oxy-hydrogen flame is very strong and homogeneous and does not shrink. For a glower of about 2 millimeter thickness and 35 a length of about 2 centimeter, the starting voltage of about from 275 to 300 volts suffices and when the glower becomes conductive this voltage drops to about 250 volts for continuous operation. Mixtures of aluminum 40 oxid or topaz (which is an aluminum fluo-silicate) with a few per cent. of either calcium, thorium, yttrium, etc., oxids, which lower the starting voltage and at the same time preserve the melting point of or raise 45 it above that of aluminum oxid may be built up in the oxy-hydrogen flame in this general manner.

Other methods of producing the glowers 50 may be employed. I have for instance, obtained very good results by mixing the aluminum oxid with a suitable binder and squirting it through a die by the usual methods employed. The filament or glower thus obtained is then roasted to remove the binder 55 and shrunk into a homogeneous mass by subjecting it to extremely high temperatures. This rod of aluminum oxid is then flashed in the vapors of an aluminum silicate, in the manner just described, in order to deposit 60 thereon a thread or group of threads of the new compound which is a complex aluminum silicate.

Instead of obtaining a thread of a better 65 conducting substance upon the glower by flashing it, the alumina and the better con-

ducting substances, as, for example, an aluminum silicate or yttrium oxid may be squirted separately but simultaneously through a properly constructed die, thus obtaining a strong body of alumina with a fine line of the other substance embedded in or alongside of it. This rod is then baked at high temperatures by any of the well-known methods.

The accompanying Figures 1 and 2 show a 75 glower constructed in accordance with my invention. Fig. 3 is a diagram illustrating the distribution of energy. Fig. 1 shows a glower consisting of a thin thread B of the better conducting material, for example, feldspar, joined to the more refractory and less conducting base of aluminum oxid A. Fig. 2 is a cross section of Fig. 1.

The principle on which my glower operates is as follows: There are two conditions 85 to be fulfilled in order to attain a high luminous efficiency in solids which are electrically non-conducting at room temperature (20° C.) but are conducting at high temperatures (1200° to 1500°) and these conditions 90 are (1) the use of a thin layer of a substance which can be operated near its melting point, (which melting point must be high) without evaporation and (2) as such a thin layer cannot be so operated without melting 95 and forming an arc, the combination of this material with a support, in such a manner that the infra red emission spectrum of the combination remains discontinuous even at the highest operating temperatures. The 100 glower of the present invention fulfils these two conditions, inasmuch as the thin thread or film of better conducting material which is a new compound of unknown composition 105 is operated near its melting point, while the 110 main body of the glower acts as a support, and the material of that support is chosen 115 with a view of having its emission spectrum very discontinuous and very much suppressed in the infra red. Both the main body of the glower and the thread along its side emit a banded spectrum. It is to be understood that the thread is the principal source of light and that the main body is but little more than a support. Of course, it 115 emits some light and the banded spectrum prevents it from emitting much heat, thus preventing a dissipation of energy, which then goes toward raising the temperature 120 and light emission of the thread.

It is thus possible to operate such a thread near its melting point, which cannot be done with any ordinary filament or glower, as the latter, when it is operated so close to its melting point, sags, melts and breaks.

In order to illustrate more clearly the physical property of the glower of my invention, I give, in Fig. 3, curve a, the distribution of energy in the spectrum which one obtains from an ordinary glower, when it is 130

highly incandescent. In curve *b* I give the distribution of energy in the spectrum of a glower of my invention, when it is operated at high incandescence. It is, of course, understood that the indentations in curve *b* vary somewhat with the composition of the glower. For example, the band at about  $3\mu$  ( $\mu=.001$  m m) is owing to silicates. However, under all conditions curve *b* is always deeply indented.

Now, as in any ordinary indicator diagram, such as one obtains in the expansion of steam in an engine cylinder, the area under the curve *a* and the horizontal axis of reference is a measure of the energy put into the glower. Similarly the area under the curve *b* is a measure of the energy which must be put into the glower of my invention, in order that it will emit the same amount of energy as in curve *a*, in the "visible spectrum." The area between the curves *a* and *b* gives the amount of energy that is wasted (as useless infra red radiations not affecting the eye) in a glower of type *a* when it emits the same amount of energy in the "visible spectrum" as does a glower of my invention.

The processes set forth above in the preparation of the glower cause the latter to have certain physical characteristics, that is, a marked banded emission spectrum in the infra red which is not possible to obtain by methods heretofore described.

I claim as my invention:

1. The process for the manufacture of glowers for incandescent lamps, which consists in providing a rod of aluminum oxid with terminals of aluminum silicate and allowing an electrical spark discharge to take place between the terminals.

2. The process for the manufacture of glowers for incandescent lamps, which consists in providing a rod of aluminum oxid with terminals of an alkali metal aluminum silicate and allowing an electrical discharge to pass between them.

3. The process for the manufacture of glowers for incandescent lamps, which consists in attaching terminals of sodium aluminum silicate to a rod of aluminum oxid and passing an electrical discharge between them.

4. The process for the manufacture of complex aluminum silicates, which consists

in providing a rod of aluminum oxid with terminals of aluminum silicate and allowing an electrical discharge to take place between said terminals for the purpose of forming a layer of the new compound substantially as described.

5. The process for the manufacture of complex aluminum silicates by passing an electric discharge over the rod of aluminum oxid, in a vapor of aluminum silicate for the purpose of forming a layer of the new compound upon the rod of aluminum oxid.

6. A glower for incandescent electric lamps consisting of a main body of aluminum oxid and a thin band of a compound composed of aluminum silicate and aluminum oxid.

7. A glower for incandescent electric lamps consisting of a compound of aluminum oxid and aluminum silicate.

8. A glower for incandescent electric lamps consisting of a compound of aluminum oxid and an alkali metal aluminum silicate.

9. A glower for incandescent lamps consisting of a compound of aluminum oxid and potassium aluminum silicate.

10. A glower for electric lighting apparatus composed of a main body of aluminum oxid and a thread of complex aluminum silicate attached thereto, the combination having the physical property of emitting a banded spectrum in the infra red, when heated to or above 1800 to 2000 degrees centigrade.

11. A glower for incandescent lamps composed of complex aluminum silicate, which has the physical property of emitting a banded spectrum in the infra red when heated above 1800 degrees centigrade.

12. As a new article of manufacture, a glower composed of second class conductors having the physical property of emitting a banded spectrum in the infra red, at or above 1800 degrees centigrade.

Signed at Washington in the District of Columbia this seventh day of July A. D. 1908.

WILLIAM WEBER COBLENTZ.

Witnesses:

FLORA RAYMOND,  
L. L. BOYD.